

## UNITED STATES PATENT OFFICE

2,113,754

## LUBRICATING COMPOSITION

John C. Zimmer, Hillside, and Arnold J. Morway, Roselle, N. J., assignors to Standard Oil Development Company, a corporation of Delaware

No Drawing. Application June 6, 1935,  
Serial No. 25,308

7 Claims. (Cl. 87—9)

The present invention relates to improvements in oils and specifically to improvements in the lubricating properties of oils and greases. The invention will be fully understood from the following description of the composition and the methods of manufacturing same.

Hydrocarbon lubricants are not characterized by an exceptionally high degree of "oiliness", and in recent years it has been found desirable to 10 find methods for increasing the oiliness or lubricity of these materials. Various substances have been added to the oils, such as fatty acids, their esters, chlorinated materials and the like; but most of such materials are undesirable in one or more respects—although they may produce a marked improvement in one or more different characteristics. There has been a steady search for materials which would improve the oiliness without increasing carbon-forming tendency, 15 oxidation rate, sludging rate, corrosion and the like.

The principal feature of the present invention is the use of a new class of organic acid compounds in lubricating oils. These materials are 20 found to be superior in aggregate of their properties to the general class of organic esters. No reason is apparent for their superiority, and the inventors content themselves with noting the fact without explanation thereof.

The particular class of compounds to which the present invention relates are compounds of 25 furoic acid, or pyromucic as it is sometimes called, the formula being  $C_4H_3OCOOH$ . The acid itself is included as well as the various alkylated 30 or hydrogenated acids, but the esters of these acids are preferable to the acids themselves.

Among the esters, the monohydric aliphatic 35 alcoholic esters are the best, such as methyl, ethyl, propyl, butyl, and amyl, but higher alcohol esters such as lauryl, cetyl, octadecyl and oleyl 40 are quite satisfactory. While the foregoing esters are most useful, it should be understood that dihydric or polyhydric aliphatic esters may be used, such as glycol or glycerol esters and the 45 esters of aromatic alcohols such as phenol, cresol and benzyl furoates.

The various compounds and particularly the 50 esters are to be used in proportion of  $\frac{1}{2}$  to 10% by weight of the oil, although usually 2% is sufficient. Various other ingredients may be added, depending on the particular use to which the oil is intended; for example, pour inhibitors, dyes, 55 thickeners, soaps, oxidation inhibitors and the like. The esters are also suitable additions to

gasoline and give it excellent upper cylinder lubricating properties.

The oil itself may be of a particular type, as for instance, derived from a paraffinic or naphthenic crude refined by the ordinary methods, such as acid or alkali treatment, solvent extraction, hydrogenation, destructive hydrogenation or the like.

While the furoic esters are of importance in 10 liquid lubricants, they are also important constituents for greases. Their function is not only limited to increasing the load bearing capacity, but also have a very desirable plasticizing effect on heavy high melting waxes which may be naturally present in the oil or may be added. These 15 greases may be made in the usual manner with soda or potash, and the furoic ester is preferably added after the grease is formed.

The effect of the furoic esters is particularly 20 desirable in producing "so-called" reversible calcium greases. Calcium greases, as made at the present time, contain small amounts of water which is essential to a proper grease consistency, and in consequence when the grease is melted, 25 the water is lost and the grease structure is broken down, leaving a hard, solid, non-greasy mixture. Such greases are "irreversible". In making "reversible" lime greases, that is, greases which can be melted and resolidified without losing the grease structure, sulfonic compounds, 30 especially the salts of mahogany sulfuric acids derived by the treatment of mineral oils with concentrated or fuming sulfuric acid, must be added to the grease, along with or in lieu of water, and a high melting wax, such as petro- 35 latum, Montan, carnauba or candellia wax. Such compounds may be varied considerably in their properties of ranging the proportion of ingredients but they are very satisfactory, and are capable of being melted and re-melted without 40 permanent loss of grease structure, which is due to the combined action of the sulfonates, the wax and the plasticizing action of the furoic esters. The amount of wax may vary from say 5 to 20%, 45 while only small amounts of the sulphonates and furoates—say  $\frac{1}{2}$  to 10% are necessary—usually 2 to 5% is best. It will be understood that 50 another calcium soap is present as well as lubricating oil. Water may be present originally for  $\frac{1}{2}$  to 1%, and glycerine, depending on whether fats or fatty acids are used in making up the calcium soap.

The following examples are given to illustrate 55 the method of producing the above-described compositions and their properties:

The oil selected for the following tests was an S. A. E. 20 lubricating oil, and to it was added 2% butyl furoate. One sample of the oil was used as a blank for comparison with other samples which 5 contained the addition agent.

The following table shows the comparison of the oxidation rate:

*Example I*

| 10                                    |  | Oxidation rate @ 200° C.<br>cc./oxygen/10 cc. sample/15 minutes |
|---------------------------------------|--|-----------------------------------------------------------------|
| Hydrocarbon lubricating oil           |  | 62-93-56                                                        |
| Hydrocarbon oil plus 2% butyl furoate |  | 23-42-40-35                                                     |

15 This action of the ester is remarkable in that the addition of most of the esters tends to increase the oxidation rate.

The oxidation rate of the oil was determined by passing oxygen in a closed cycle at a constant 20 rate, so as to bubble through a container holding exactly 10 cc. of the sample. This was maintained at a temperature of 200° F., and at intervals of 15 minutes the amount of oxygen absorbed 25 was determined by measuring the remaining oxygen.

*Example II*

The samples used in Example I were then tested for corrosion of bearings of several different 30 compositions. These data are as follows:

| 35                                    | Lubricating oil | Cd-Ag bearings<br>Hours of test |     |     |     |
|---------------------------------------|-----------------|---------------------------------|-----|-----|-----|
|                                       |                 | 50                              | 100 | 200 | 300 |
| Hydrocarbon oil                       |                 | 0                               | 1   | 1   | 1   |
| Hydrocarbon oil plus 2% butyl furoate |                 | 0.4                             | 0.6 | 0.9 | 0.9 |

| 40                                 | Lubricating oil | Cd-Ag bearings<br>Hours of test |     |     |     | Cd-Ni bearings<br>Hours of test |     |     |     |
|------------------------------------|-----------------|---------------------------------|-----|-----|-----|---------------------------------|-----|-----|-----|
|                                    |                 | 50                              | 100 | 200 | 300 | 50                              | 100 | 200 | 300 |
| Hydrocarbon oil                    |                 | 1                               | 2   | 2   | 2   | 0                               | 1   | 37  | 172 |
| Hydrocarbon oil + 2% butyl furoate |                 | 0.2                             | 0.4 | 0.4 | 0.5 | 1.1                             | 1.2 | 1.3 | 1.3 |

50 The foregoing tests were carried out in a strictly comparable manner at a temperature of 210° F. and show that the butyl furoate was substantially less corrosive than the oil itself in all three cases. The figures represent loss in milligrams.

*Example III*

The samples used in the tests were then subjected to a further test to show their oiliness 60 characteristics on the Mougey machine described by Mougey and Almen in the International Petroleum News. The first test showed a bearing combination of aluminum and steel with hydrocarbon oil as follows:

| 65                                   | Lubricating oil | Lbs./sq. in. | Friction |
|--------------------------------------|-----------------|--------------|----------|
| Hydrocarbon oil                      |                 | 18,000       | Sheared  |
| Hydrocarbon oil + 2% butyl furoate   |                 | 25,000       | 18       |
| Hydrocarbon oil + 1% butyl furoate   |                 | 25,000       | 38       |
| Hydrocarbon oil + 1/2% butyl furoate |                 | 25,000       | Sheared. |

70 From the above it will be seen that the addition of ester produced a very substantial increase in the oiliness and load bearing capacity of the oil.

*Example IV*

As an example for the preparation of a reversible grease, the following information may be of assistance:

About 69 1/2% by weight of a red machine oil having a viscosity of 300 seconds Saybolt at 110° F. is placed in a fired kettle, and ten parts of high-melting petrolatum wax (180° F. melting point) is then added, and the mass is heated to about 200° F. while thoroughly agitated. At this point about fifteen parts of horse fat is added and the temperature is raised to about 350° F., at which point the amount of hydrated lime requisite for saponification is added at that temperature. The product was then cooled to about 250° F., and about 2% of calcium sulfonate added. This material is derived from the mahogany acid obtained by sulfonation of petrolatum distillates. It was worked carefully into the composition by agitation, and when this was completed the resulting product was cooled to about 200° F. and 2% of butyl furoate was added. The product was again cooled and the grease structure obtained by the usual methods employed in the preparation of lime soap greases. The final material had the following compositions:

|                                       | Percent |
|---------------------------------------|---------|
| Red machine oil                       | 69 1/2  |
| Petrolatum wax, 180° F. melting point | 10      |
| Lime soap                             | 15      |
| Calcium sulfonate                     | 2       |
| Butyl furoate                         | 1       |
| Water                                 | 1/2-1   |
| Glycerine                             | 1 1/2   |

The grease had a penetration of approximately 270 at 77° F., and on heating to 300° F. with loss of water was reduced to a thick fluid state. On cooling the product resolidified into a smooth, 40 uniform grease. The A. S. T. M. penetration of the resolidified grease was 250-275 at 77° F., and it was found that melting and remelting any number of times did not substantially change the quality of the grease.

45 For comparison, a grease made up in substantially the same way which did not contain the butyl furoate showed a similar penetration of about 270 before melting. After melting this dropped to about 100-125, showing that the material had become much harder and had in fact lost its grease properties.

*Example V*

To an aviation gasoline having an initial boiling point of 110° F. and end point of 280° F. is added 55 1% of butyl furoate, which dissolved readily. The operation of the engine was smoother when this fuel was used than when the fuel was used in the absence of the furoate.

The present composition and methods of manufacture are not limited to any theory of the function of any of the ingredients, nor to any particular ingredient which may have been used 60 for illustrative purposes, but only to the following claims, in which it is desired to claim all novelty inherent in the invention.

We claim:

1. An improved lubricant comprising a hydrocarbon oil and a neutral ester of furoic acid.
2. Lubricant according to claim 1 in which a neutral aliphatic alkyl ester of furoic acid is used.
3. Lubricating oil according to claim 1 in which

a neutral aliphatic monohydric alkyl ester of furoic acid is used.

4. An improved lubricant comprising a hydrocarbon lubricating oil and about  $\frac{1}{2}$  to 10% of a monohydric alkyl ester of pyromuic acid.

5. A solid lubricant comprising hydrocarbon lubricating oil, soap in proportion to solidifying the same, and a neutral ester of furoic acid.

6. A composition according to claim 5, comprising lime soaps, lubricating oil, and a neutral ester of furoic acid.

7. A composition according to claim 5, comprising a lubricating oil, high melting wax, a 5 calcium soap of a sulfonic acid, and butyl furoate.

JOHN C. ZIMMER.  
ARNOLD J. MORWAY.